

April 18, 1933.

M. HAGEDORN

1,904,221

PROTECTIVE LAYER ON PHOTOGRAPHIC FILMS

Filed April 25, 1927



Max Hagedorn Inventor

by Byrnes, Townsend & Brickestein

his Attorneys.

## UNITED STATES PATENT OFFICE

MAX HAGEDORN, OF DESSAU IN ANHALT, GERMANY, ASSIGNOR, BY MESNE ASSIGNMENTS, TO AGFA ANSCO CORPORATION, OF BINGHAMTON, NEW YORK, A CORPORATION OF NEW YORK

## PROTECTIVE LAYER ON PHOTOGRAPHIC FILMS

Application filed April 25, 1927, Serial No. 186,567, and in Germany May 1, 1926.

One applies a protective layer to the back surface of a photographic film for several purposes; for instance for preventing the film from rolling up during development, 5 fixing and drying, for making the film less liable to damage, making it softer and better adapted to slide, which is of particular importance in the cinematograph film; for protecting the film against electric discharges 10 which are liable to occur owing to the electrical excitation of the film, it may be by movements in the cinematograph apparatus, for minimizing the alteration in length and breadth of the film owing to the effect of 15 atmospheric moisture.

For these purposes protective layers of various kinds have been suggested, for example varnishes, resins, gelatin, individual cellulose esters and ethers, either alone or 20 with addition of electrolytes, substances which are hygroscopic or diminish the surface tension or friction of the film. Another proposition has been that the back surface of the emulsion carrier should be varied in 25 its composition by treating it with solvents, with or without the addition of electrolytes or substances which are hygroscopic or diminish the surface tension or the friction of the surface.

30 In order to lend to the protective layer the properties desired for the particular purposes, the layer has been made up of advantageously mixed substances which are more or less foreign to the emulsion carrier.

35 As contrasted with this practice a protective layer which does not consist of a mixture but is a chemical individual compound of the properties required for the purpose would be a technical advance.

40 The present invention consists of a protective layer made of cellulose derivatives other than nitroacetate soluble in organic solvents and containing several different radicles as substituents, particularly radicles of more than one acid or besides 45 ether groups radicles of acids. Such compounds may be obtained from cellulose derivatives having still esterifiable hydroxyl groups, particularly from mono-esters, di- 50 esters, mono-ethers, di-ethers or mixtures of

such compounds, swollen or dissolved in organic solvents by treating them, preferably in the presence of a substance promoting the esterification, with functional derivatives of inorganic or organic acids, for instance 55 their esters, chlorides, amides, anhydrides or mixed anhydrides.

According to the desired effect a suitable cellulose derivative of the indicated kind is selected for the particular case, which presents no difficulty, since a large number of these compounds having correspondingly different properties are available. For example, if a film having a high capacity for sliding and small shrinkage is required there 60 may be used cellulose-acetate-stearate as protective layer. The same effect has a protective layer made from cellulose-ethyl-ether-stearate. When protection against electric 65 discharges is in question the layer may consist of cellulose-ether-phosphate or cellulose- 70 acetate-phosphate.

In carrying out the invention a solution of the said cellulose derivates containing several different radicles as substituents is applied to the photographic film, particularly 75 to the back surface of such a film.

The following examples illustrate the invention without limiting it:

Example 1.—60 grams of cellulose-acetate- 80 phosphate are dissolved in 3750 cc. of acetone and 1600 cc. of water, with addition of 300 cc. of glycol - mono - methyl - ether - acetate. The layer produced by applying this solution in the known manner to the back surface 85 of the film imparts good protection against electric discharge.

Example 2.—For producing a protective layer on the back surface of the film there is used a 1 per cent solution of cellulose-ethyl-ether-stearate or cellulose-acetate-stearate in a mixture of 1 part of alcohol, 3 parts of benzene and 2 parts of acetone. This layer greatly diminishes the resistance of the film to sliding in the cinematograph apparatus. 90

The aforesaid solutions may contain still other additions remaining in the dry layer.

The accompanying drawing shows on an enlarged scale in section a film provided with a protective layer according to the present 100

invention. It is to be understood that the invention is not limited to films embodying the especial ratio of thicknesses of layers represented in this drawing.

5 Having now particularly described and ascertained the nature of my said invention and in what manner the same is to be performed, I declare that what I claim is:—

10 1. A photographic film with a protective layer on its back surface, said layer comprising a compound of the group consisting of cellulose-ether-stearate, cellulose-ether-phosphate, cellulose - acetate - stearate, and cellulose-acetate-phosphate.

15 2. A photographic film with a protective layer on its back surface, said layer consisting of cellulose ether-phosphate.

20 3. A photographic film with a protective layer on its back surface, said layer comprising a cellulose derivative of the group consisting of cellulose mixed esters of two fatty acids, cellulose mixed esters of one fatty acid and phosphoric acid, cellulose ether esters of fatty acids, and cellulose ether esters of 25 phosphoric acid.

In testimony whereof I affix my signature.  
MAX HAGEDORN.

30

35

40

45

50

55

60

65